

## UNITED STATES PATENT OFFICE

1,975,671

PROCESS OF MANUFACTURING LEATHER  
AND PRODUCT USED IN CONNECTION  
THEREWITHCharles G. Shaw, Huntsville, Ontario, and Jacques  
Hoffman, Toronto, Ontario, CanadaNo Drawing. Application June 3, 1930, Serial No.  
459,104. In Canada November 29, 1929.

## 1 Claim. (Cl. 91—68)

This invention relates to a process of applying coating materials to sole leather and particularly to the application of such coating materials prior to the completion of the filling of the leather and the mechanical operations of smoothing the leather.

In our co-pending application, Serial No. 459,103, filed June 3, 1930, we have described a method of applying coating materials to sole leather after the filling and tanning steps. Previous to our discoveries in connection with the application of coating materials, the adhesion of such materials to the grain of sole leather was such that when the leather was subjected to such operations as drumming with fillers in a stuffing drum, after having been coated, the coating would not adhere and would be mutilated and destroyed by such operations. Furthermore, when leather, which had previously been filled with such materials as wax, resin, oil, tanning extract, sugar and the like, was coated or painted for the purpose of rectifying the unpleasant color caused by the filling, any coating so applied would be removed by subsequent operations in the shoe factory, thus exposing the unpleasant color beneath.

In the application of permanent waterproof coatings on sole leather and particularly with reference to the adhesion of these coatings, there are two principal controlling factors, in addition to the composition of the coating material itself. During our experimental work, the repeated failures of the coatings to adhere were at first attributed to the tanning materials and fillers lying upon the surface of the leather. These materials and fillers were almost entirely of a water soluble nature and their presence was considered responsible for the failure of the adhesion when the coated leather was re-soaked. A great many tests were carried out in applying coatings to leather from which the fillers had been carefully cleansed from the surface. Those tests proved that neither the quantity of filler nor the composition of the filler had much effect upon the adhesion of the coating. We then discovered that the physical properties of the surface of the leather ordinarily constituted the controlling factor in the adhesion of a coating material to sole leather which was reasonably free from an excess of fillers. Coatings for sole leather were made adherent by applying the coating to the leather in the absence of the glossing effect of the setting out and finishing operations, which latter operations had a tendency to compact the surface or hyaline layer of the leather and form of it a filter into which the constituents of the coating material would not penetrate. We then found that if the sole leather was previously completely saturated with fillers such as wax, grease or water-soluble fillers,

the adhesion would then be controlled by the quantity and the nature of the filling ingredients.

We have now discovered that coating materials may be applied to leather before the completion of the filling process and even in some cases before the completion of the tanning operations. In fact, the coating materials may be applied and the leather may be subsequently saturated, or filled as desired, with any suitable material, and with the coating applied so as to adhere properly to the leather fibre or substance itself, the subsequent filling operation having no effect upon the adhesion.

One of the principal objects of this invention is to incorporate into the leather an extraordinary amount of tanning and/or filling materials without interfering with the adhesion of a coating material applied for the purpose of rectifying the color of the leather so produced.

Another object is to eliminate the cost of re-finishing the soles after the shoes have been made.

A further object is to provide a product in which the applied coatings may be both oil proof and water-proof, but which product will nevertheless permit the rapid soaking of the leather through the coating.

A still further object is to provide a product which will enable the manufacturer of sole leather to disregard color in the selection of his tanning and filling materials and also the extent to which many fillers may be incorporated without making the leather unsightly.

Our invention consists essentially in the process of applying one or more coating compositions, either clear or pigmented, to the grain surface of sole leather prior to the completion of the filling operation, or even prior to the completion of the tanning operation. When filling materials such as corn sugar, tanning extract, oil, wax, resin, asphaltum, and the like, are incorporated into the leather in large quantities, prior to the coating process, the adhesion of the coating to the leather is seriously interfered with as the bonding, in such cases, is more apt to be to the filling substance rather than to the leather substance.

In carrying out our invention, the following procedure may be employed. The leather is taken from the tan liquor and preferably washed to remove water-soluble substances from the surface of the leather. It is then dried so as not to exceed about forty percent moisture by weight. It may be stated that the moisture content is determined by the constituents of the coating composition, but, generally speaking, the leather should be dried to a point where proper adhesion of the first coating takes place easily. The leather is now ready for the coating compositions which are preferably applied by means of an air spray gun. The composition of the priming coat con-

sists of a cellulose ester such as nitro cellulose 5 parts, castor oil 3 parts, boiled linseed oil 1½ parts, ethyl acetate 25 parts, amyl acetate 8 parts, and toluol 40 parts. This composition in approximately the proportions mentioned is applied to the leather and allowed to air dry for about one hour. A coating of finishing composition may now be applied in a similar manner consisting of raw sienna 10 parts, pyroxalin 7 parts, butyl acetate 20 parts, ethyl acetate 20 parts, butyl lactate 3 parts, toluol 20 parts, and castor oil 6 parts. This finishing coat is allowed to dry and the leather may then be saturated and filled by drumming in a mixture such as the following:

|    |                                                                                                                |       |
|----|----------------------------------------------------------------------------------------------------------------|-------|
| 15 |                                                                                                                | Parts |
|    | Corn sugar                                                                                                     | 20    |
|    | Water                                                                                                          | 10    |
|    | Magnesium sulphate                                                                                             | 10    |
| 20 | Stearine                                                                                                       | 20    |
|    | Paraffine wax                                                                                                  | 20    |
|    | Asphalt                                                                                                        | 15    |
|    | Varnolene a petroleum distillate used as a turpentine substitute having a boiling range from about 310 to 415° | 15    |
| 25 | Sulphonated fish oil                                                                                           | 5     |

This drumming operation is preferably carried out at a temperature between 100° F. and 130° F. The surface of the leather is then freed of excess filling composition by a setting out operation on the grain side and at the same time spraying the grain surface of the leather with water warmed to not over 100° F. for vegetable tanned leather and not over 200° F. for chrome tanned leather. The coating on the grain surface is then sponged with a substance such as naphtha to remove the filling material from the surface. An additional coating of a finishing composition similar to that mentioned above is then applied as before and the leather is afterwards thoroughly dried and compacted in the ordinary manner of treating sole leather.

While we prefer to perform the filling operation in the manner above described, the filling materials may be incorporated into the leather by a process of immersion or by treating the leather in a vacuum in the presence of the fillers or by subjecting the leather which is submerged in the fillers to pressure within a suitable vessel. It should be observed that the coating will not adhere satisfactorily to the leather if, in drying from the tan liquors, it becomes excessively oxidized or "liquor-stained", or if excessive amounts of water or water-soluble substances are present.

While we have found it preferable to use a priming coat and a finishing coat consisting of the ingredients in the proportions above stated, we do not restrict ourselves to such proportions and we desire to include within the scope of our invention equivalent ingredients as modifications thereof. We do, however, find it essential that the coating compositions should contain either a cellulose ester or a resin, preferably a synthetic resin. The compositions may, if desired, contain suitable pigments or coloring matter.

These compositions should preferably be applied by means of an air spray gun so as to prevent permanent plugging of the hair holes in the leather, thus facilitating the rapid penetration of tanning agents or liquid matter into the pores or hair holes of the leather. However, the compositions may be applied in any manner as by pour-

ing or swabbing, in which case the hair holes should be re-opened by mechanical working of the leather. The process is intended to be applied to sole leather which has not been completely filled and which may be partially or completely tanned. After the application of the first coat, the leather may be filled with any suitable filling material, excepting those fillers which exert a softening or solvent action upon the coating. Any stains consequent upon the filling of the leather may be covered over by the application of a further coat of finishing compound containing a pigment or coloring matter. In this case, the surface of the first coat should be cleansed of foreign matter to facilitate the adhesion of one coat to another.

Filling materials which are commonly incorporated into leather are either water-soluble, or of a greasy or waxy nature. Leather into which such substances have been largely incorporated, does not lend itself to coating processes as readily as unfilled leather, in which latter case the adhesion of the coating materials is more to the actual leather fibres and less to the filling or tanning materials.

By means of this invention, a product may be produced having a uniform coating of any desired color, regardless of the type of tanning or filling material employed. Such leather is particularly suitable for loggers' boots, which may be made impervious to water; to Goodyear insoles, which may be made exceedingly tough by stuffing with wax or the like so that they will not stain hosiery; to sport shoes, which may be made very flexible by impregnation with gums; to chrome leather, which may be given the appearance of oak tanned leather; and to many other types of leather useful for various purposes.

By this process a perfect adhesion of the coating to the leather is produced, so that it will withstand the action of subsequent drum stuffing, or other filling processes, and will not be damaged by various conditions to which such leather is subjected. Materials such as rubber and asphalt may be used as fillers for the leather to increase wear resistance, where formerly such materials could not be employed. Moreover, larger percentages of oil may be employed as a filling material to nourish and preserve the leather fibre without producing unsightly colors or stains.

Finally, as a result of our process, a very rapid penetration of the fillers through the coating takes place because when the hair holes are open and unclogged, the fillers or tanning liquors pass through these hair holes into the leather and this is a great advantage in a leather manufacturing process. Although this process has been described as being applied particularly to sole leather, it may be applied to other types of leather.

Having thus described our invention, what we claim is:

A process of manufacturing sole leather which includes the steps of applying one or more permanently adhesive waterproof coatings, containing such a material, as cellulose ester, to the surface of sole leather prior to the completion of the filling operation, rupturing the coating materials bridged over the hair holes of the leather and then subjecting the leather to the filling and finishing operations.

CHAS. G. SHAW.

JACQUES HOFFMAN.